

May 3, 1927.

1,627,070

E. WEINTRAUB

METALLIC VAPOR DEVICE

Filed Dec. 14, 1923

Fig. 1.



Fig. 2.



Fig. 3.



INVENTOR

Ezechiel Weintraub

BY

Pennie, Davis, Marvin & Edmonds

ATTORNEY

## UNITED STATES PATENT OFFICE.

EZECHIEL WEINTRAUB, OF NEUILLY-SUR-SEINE, FRANCE.

## METALLIC VAPOR DEVICE.

Application filed December 14, 1923. Serial No. 680,691.

In metallic vapor devices such as mercury vapor lamps and rectifiers, the familiar continuous movement of the so-called cathode spot on the surface of the mercury cathode 5 is an objectionable characteristic—partly on account of the fluctuating light emitted in the case of lamps, and partly on account of the irregularity of current flow resulting therefrom in the case of rectifiers. Furthermore, it has been found that the minimum current on which these devices will 10 operate is very considerably increased on account of this phenomenon.

For the purpose of fixing the cathode 15 spot, it has heretofore been proposed to affix to the mercury cathode an emergent pointed stud or equivalent element made of either platinum or copper. These metals will function as intended to fix the cathode spot, 20 but have been found commercially impracticable on account of the facts that platinum is appreciably disintegrated by the ionic bombardment occurring in the operation of the device and copper dissolves in the 25 mercury. In each instance the disintegrated metal forms a film-like coating on the walls of the receptacle to which the condensed mercury adheres. This coating is electrically 30 conductive and, being formed on the insulating parts of the apparatus, is likely to cause short-circuits between the electrodes. It also happens that the cathode spot is often formed upon this coating, thereby 35 causing irregularities in operation and frequently cracking the glass receptacles on account of high temperature.

I have found by experiment that certain metals having the properties of high refractivity and high density are free from 40 the above-mentioned objectionable characteristics of platinum and copper, in that they do not become disintegrated by the ionic bombardment and do not dissolve in the mercury. The metals which I have 45 found to be most particularly adapted for this purpose are tungsten and molybdenum. Both of these metals are classified in the sixth group of Mendeleef's periodic table. Molybdenum has a specific gravity of 9.01 50 and tungsten of 19.6. The melting points of both these metals are above 2000° C.

Another metal which may be utilized for the same purpose is tantalum. This latter metal is classified in the fifth group of Men-

deleef's periodic table, and has a specific 55 gravity of 14.49 and a melting point above 2000° C.

From the foregoing it will be seen that the metals which have been found to be operative for the purpose set forth and free 60 from the objectionable characteristics of platinum and copper may be defined as being included in the combined fifth and sixth groups of the periodic table and having specific gravities at least as great as that 65 of molybdenum and a melting point greater than 2000° C.

Not only may these metals be used individually for the purpose of this invention, 70 but certain of their alloys may also be successfully employed—due regard being had for the essential properties of high density and refractivity, as well as for the practical necessity of selecting an alloy which may be satisfactorily worked.

With reference to the accompanying drawing, Figs. 1, 2 and 3 show fragmentary cross-sectional views of mercury vapor devices illustrating three alternative embodiments of the invention.

In each figure A is a mercury cathode, B is a glass receptacle, and C is an auxiliary anode for starting the device in operation. D, E and F are the electrode elements in accordance with this invention.

In Fig. 1, the electrode D is in the form of a rod, the upper end portion of which projects beyond the surface of the mercury cathode.

In Fig. 2, the electrode E is made of wire 90 or rod and its upper end portion is spirally formed.

In Fig. 3, the upper end portion of the electrode F has the form of a cylindrical tube.

The particular form of electrode employed is inconsequential—those illustrated being merely by way of example. For handling small currents, a rod electrode as in Fig. 1 is generally employed, while for large currents either a spiral or cylindrical electrode as in Figs. 2 and 3 is used.

In rectifiers not provided with artificial cooling means and intended to handle up to 40 amperes, it is advisable to allow from 105  $\frac{3}{4}$  to 1 millimeter of contact line per ampere between the mercury and the electrode element at the surface of the mercury.

When artificial cooling is provided, much less than 1 millimeter contact line per ampere need be provided.

In a big iron rectifier which has been constructed in accordance with this invention, it has been found that a cylindrical molybdenum electrode will successfully fix the cathode spot when the device is passing over 300 amperes. Such an electrode provides about 157 millimeters contact line. This is slightly over  $\frac{1}{2}$  millimeter per ampere.

In mercury vapor devices in which the cathode spot is not fixed, it has been found that the minimum operating current is approximately 3 amperes. When the cathode spot is rendered stationary in accordance with the present invention, the minimum operating current which may be realized is reduced to approximately 1 ampere. This is obviously a very distinct advantage.

I claim:

1. In a mercury vapor device including a mercury cathode, means for fixing the cathode spot comprising an electrode element in contact with said mercury cathode, said electrode comprising metal classified within the combined fifth and sixth groups of the Mendeleef periodic system and having a specific gravity at least as great as that of molybdenum and not greater than that of tungsten and melting point above 2000° C.

2. In a mercury vapor device including a mercury cathode, means for fixing the cathode spot comprising an electrode element in contact with said mercury cathode, said electrode comprising metal classified in the sixth group of the Mendeleef periodic system and having a specific gravity at least as great as that of molybdenum and melting point above 2000° C.

3. In a mercury vapor device including a mercury cathode, means for fixing the cathode spot comprising an electrode element in contact with said mercury cathode, said electrode comprising metals classified

within the combined fifth and sixth groups of the Mendeleef periodic system and having specific gravities at least as great as that of molybdenum and melting points above 2000° C.

4. A mercury vapor device including a mercury cathode, means for fixing the cathode spot comprising an electrode element in contact with said mercury cathode, said electrode comprising metals classified in the sixth group of the Mendeleef periodic system and having specific gravities at least as great as that of molybdenum and melting points above 2000° C.

5. In a mercury vapor device including a mercury cathode, means for fixing the cathode spot comprising a tungsten electrode element, said element being in contact with said mercury cathode.

6. In a mercury vapor device including a mercury cathode, means for fixing the cathode spot comprising an electrode element in contact with said mercury cathode, said electrode comprising tungsten and molybdenum and having a specific gravity at least as great as that of molybdenum and melting point above 2000° C.

7. In a mercury vapor device including a mercury cathode, means for fixing the cathode spot comprising an electrode element in contact with said mercury cathode, said electrode being made of an alloy comprising tungsten and molybdenum and having a specific gravity at least as great as that of molybdenum and melting point above 2000° C.

8. In a mercury vapor device including a mercury cathode, means for fixing the cathode spot comprising an electrode element in contact with said mercury cathode, said electrode being made of an alloy comprising tungsten, molybdenum and tantalum and having a specific gravity at least as great as that of molybdenum and melting point above 2000° C.

In testimony whereof I affix my signature.  
EZECHIEL WEINTRAUB.